# EUROPEAN PATENT SPECIFICATION

(11) **EP 0 296 793 B1**
(45) Date of publication and mention of the grant of the patent: **25.08.1993**
(21) Application number: 88305631.9
(22) Date of filing: 22.06.1988
(51) Int. Cl.: G03C 7/36, C07C 317/22

(54) **Colour photographic silver halide materials and process**
Farbphotographische Silberhalogenidmaterialien und Verfahren
Matériaux photographiques couleurs à l'halogénure d'argent et procédé

(30) Priority: 25.06.1987 GB 8714866
(43) Date of publication of application: 28.12.1988
(73) Proprietor: EASTMAN KODAK COMPANY (a New Jersey corporation), Rochester, New York 14650 (US); KODAK LIMITED, Hemel Hempstead Herts, HP1 1JU (GB)
(72) Inventor: Clark, Bernard Arthur James, Holiport Maidenhead Berks (GB); Milner, Nigel Edgewick, Croxley Green Watford Herts (GB); Stanley, Paul Louis Reginald, Wealdstone Harrow Middlesex (GB)
(74) Representative: Baron, Paul Alexander Clifford

(56) References cited:
- US-A- 4 587 207
- PATENT ABSTRACTS OF JAPAN, vol. 9, no. 30 (P-333)[1753], 8th February 1985

## Description

This invention relates to novel acylacetanilide photographic colour couplers and photographic elements containing them.

It is well established in the photographic art that colour images may be obtained from imagewise exposed silver halide emulsions by developing them with a primary aromatic amine colour developing agent in the presence of a colour coupler. The oxidized colour developing agent formed in the areas of silver halide development couples with the coupler to form a dye. The coupler may be present in the developer solution but is normally incorporated in the sensitive photographic material.

For image dye-forming couplers to be practically useful, they must react both efficiently and at a suitable rate with oxidized developer to produce the dye. In addition, the dyes thus formed must possess acceptable hue and exhibit adequate stability over a wide range of keeping conditions.

Most of the examples of yellow image dye-forming couplers which have been used in commercial photographic products are drawn from two classes of acylacetanilide, namely pivaloylacetanilides and benzoylacetanilides. Historically, benzoylacetanilide couplers exhibit greater reactivity with oxidized developer than their pivaloylacetanilide analogues and furthermore, the extinction coefficient of their derived dyes can be greater. However, the hue of these dyes is generally deeper, and their stability on exposure to light, heat and humidity is generally poorer. Benzoylacetanilides are also more prone to crystallize either in coupler solvent or in photographic coatings.

Benzoylacetanilides have been largely superseded by pivaloylacetanilides over the last thirty years owing to the superior dye characteristics imparted by the latter. However, the present invention relates specifically to the use of benzoylacetanilides as yellow image dye-forming couplers.

European Patent Application 0126433 is largely concerned with pivaloylacetanilide couplers but three benzoylacetanilides (Compounds 4, 10 and 11) are disclosed; these compounds however do not fall within the claims of the present specification. US Patent 4,587,207 in its general description covers both pivaloylacetanilide and benzoylacetanilide but its specific disclosure is restricted to pivaloylacetanilides. Compound 17 of this patent has structural features in common with the couplers of the present invention but has the ballast group attached in a different position and has a sulphonamido group on the anilide ring. Its properties are not reported. Japanese Kokai 59-174839 also discloses similar couplers. Compound 9 of this specification also has structural features in common with the couplers of the present invention but has an alkyl ester group on the anilide ring.

A continuing need has existed for acylacetanilide yellow dye-forming couplers that, in a photographic silver halide material and process, provide excellent dye density and image contrast characteristics and provide image dyes of excellent hue and high extinction coefficients. A need also has existed for such couplers that enable improved dark keeping characteristics.

We have found that such characteristics are provided in a colour photographic silver halide element comprising a support bearing at least one photographic silver halide emulsion layer and a non-diffusible yellow dye-forming para-R-oxybenzoylacetanilide coupler that has a combination of (a) a para-hydroxyphenylsulphonylphenoxy coupling-off group in the coupling-position, (b) a chloro or trifluoromethyl group in the ortho position on the anilide moiety, and (c) a group on the anilide moiety that is selected from (i) an aliphatic hydrocarbon group that is bonded to the anilide moiety directly or through a linking group that is carbamoyl (-CONH-), sulphonate (-O-SO₂-), phosphate (-O-PO₂) or alkylene, (ii) chlorine, and (iii) trifluoromethyl; said anilide moeity having no further substituents; wherein the coupler contains at least one ballast group on at least one of the anilide and para-R-oxybenzoyl moieties; and, wherein R is an unsubstituted or substituted cyclic or non-cyclic aliphatic hydrocarbon group.

Useful non-diffusible colour couplers have the formula:
wherein
R¹ is an unsubstituted or substituted cyclic or non-cyclic aliphatic hydrocarbon group;
Y is chloro or trifluoromethyl;
Z is halogen, trifluoromethyl or -L-R² wherein
R² is an unsubstituted or substituted aliphatic hydrocarbon group,
L is a direct bond or a carbamoyl (-CONH-), sulphonate (-O-SO₂-), phosphate (-O-PO₂-), or alkylene group; and
at least one of R¹ and Z comprises a ballast group.

The benzoylacetanilide image dye-forming couplers of the invention are readily soluble in common coupler solvents and, when incorporated into a color negative photographic material, exhibit excellent dye density and contrast characteristics. Furthermore, these couplers produce dyes of excellent hue and high extinction coefficient which are stable under a wide range of conditions, particularly dark keeping which is of fundamental importance for colour negative materials.

Examples of the groups which R¹ may represent are alicyclic groups of 4 to 6 carbon atoms, and non-cyclic groups of 1-20 carbon atoms which may be substituted or unsubstituted, saturated or unsaturated, e.g. methyl, ethyl, n-butyl, n-dodecyl, n-hexadecyl, and n-undecyl.

The ballast group may form part of R¹ in which case R¹ may be an alkyl group of 10-16 carbon atoms.

The ballast can also be attached via substituent Z. In such cases, the group which links the ballast to the anilide ring has a strong influence on the solubility of the coupler in coupler solvent and also its propensity to crystallize in photographic coatings. Linking groups or atoms which have been found to confer favorable solubility characteristics on the coupler include carbamoyl, sulphonate, phosphate and alkyl. It is noted that linking groups or atoms which may give rise to coupler crystallinity problems include amide, sulphonamide and oxygen.

If the ballast is in Z, R¹ preferably contains 1-4 carbon atoms.

The aliphatic hydrocarbon groups which R² may represent can be any of the groups given as examples of R¹.

Benzoylacetanilide couplers 1 to 5 specified below are examples of couplers of the invention whose derived dyes exhibit exceptional dark/wet stability. Furthermore, these compounds display all the other characteristics required of an image dye-forming coupler for use in color negative photographic materials.
Me herein means CH₃-.

The present couplers may be prepared by methods, in themselves, known. The following synthetic procedure for coupler 8 (a coupler outside the scope of the present invention but an analogous compound) is illustrative for all the compounds of the invention.

### Preparation of coupler 8

### 1) 4-Dodecyloxyacetophenone

A stirred mixture of 4-hydroxyacetophenone (54.5g), 1-bromodecane (152.7g), potassium carbonate (83.0g) and acetone (800ml) was heated under reflux for 40 hours. The mixture was passed through a steam-heated filter and the filtrate was evaporated under reduced pressure. The residue was recrystallized from petroleum-ether (b.p. 40-60°C) to give 91.0g of product (75%).

### 2) Ethyl 4-dodecyloxybenzoylacetate

A stirred mixture of sodium hydride (25.5g, 60% mineral oil dispersion), diethyl carbonate (115.0g)and toluene (300ml) was heated to 70°C. 4-Dodecyloxyacetophenone (74.4g) in toluene (150ml) was added over 20 minutes. The stirred mixture was heated at 80°C for 2 hours, then it was cooled and carefully acidified with glacial acetic acid. The mixture was diluted with water, then it was extracted with ethyl acetate (300ml). The extract was dried over magnesium sulphate and evaporated under reduced pressure. Xylene was added to the residue and the resulting solution was again concentrated under reduced pressure to remove traces of diethyl carbonate. The residue (101.4g) was used in the next stage without further purification.

### 3) Methyl 4-chloro-3-[2-(4-dodecyloxybenzoyl)acetamido] benzoate.

A stirred mixture of ethyl 4-dodecyloxybenzoylacetate (45.6g, crude), methyl 3-amino-4-chlorobenzoate (20.0g) and xylene (400ml) was slowly distilled over 3 hours collecting about 200ml of distillate. The solution was allowed to cool and the resulting precipitate was filtered off. The product was recrystallized from acetonitrile to afford a flaky, white solid (33.9g, 60.8%).

### 4) Methyl 4-cholor-3-[2-chloro-2-(4-dodecyloxybenzoyl) acetamido]benzoate

Sulphuryl chloride (9.5g) was added over 30 minutes to a solution of the above solid (33.0g) in dichloromethane (300ml). The solution was stirred at ambient temperature for a further 1 hour before being concentrated under reduced pressure. The residue crystallized when slurried with acetonitrile. The resulting solid was recrystallized from acetonitrile to give 32.0g (91%) of pure product.

### 5) Methyl 4-chloro-3-[2-(4-dodecyloxybenzoyl)-2-(4-((4-hydroxyphenylsulphonyl))phenoxy)acetamido] benzoate

Nitrogen gas was passed through a solution of methyl 4-chloro-3-[2-chloro-2-(4-dodecyloxybenzoyl) acetamido]benzoate (22g) and sulphonyldiphenol (40g) in DMF (300ml) for 30 minutes before adding triethylamine (12.12g) dropwise with stirring. The temperature was raised to 45-50°C and maintained for 2 hours. The reaction mixture was poured into stirred 5% hydrochloric acid (300ml) and the mixture was then stirred for 1 hour. The aqueous phase was decanted and the residual gum dissolved in ethyl acetate (300ml). The organic solution was washed successively with sodium carbonate solution (300ml) and water (300ml), then it was dried over magnesium sulphate and concentrated to dryness. The resulting gum was purified by elution through a silica gel column using mixtures of ethyl acetate and petroleum-ether (b.p. 60-80°C) as the eluting solvent. The appropriate fractions were combined and concentrated under reduced pressure, and the resulting solid was recrystallized from ethyl acetate/petroleum ether to afford the required product as a white powder (14g, 46%).
HPLC analysis 99%, m.p. 153-8°C

| Elemental analysis: | | | | | |
|---|---|---|---|---|---|
| C₄₁H₄₆CℓNO₉S req: | C,64.3; | H,6.2; | C1,4.9; | N,1.8; | S,4.3%: |
| found | 64.4; | 6.0; | 4.7; | 1.8; | 4.2. |

The dye-forming couplers of this invention can be used in the ways and for the purposes that dye-forming couplers have been previously used in the photographic art.

Typically, the couplers are associated with a silver halide emulsion layer coated on a support to form a photographic element. As used herein, the term "associated with" signifies that the coupler is incorporated in the silver halide emulsion layer or in a layer adjacent thereto where, during processing, it is capable of reacting with silver halide development products.

The photographic elements can be single colour elements or multicolour elements. In a multicolour element, the yellow dye-forming couplers of this invention would usually be associated with a blue-sensitive emulsion, although they could be associated with an emulsion sensitized to a different region of the spectrum, or with a panchromatically sensitized, orthochromatically sensitized or unsensitized emulsion. Multicolour elements contain dye image-forming units sensitive to each of the three primary regions of the spectrum. Each unit can be comprised of a single emulsion layer or of multiple emulsion layers sensitive to a given region of the spectrum. The layers of the element, including the layers of the image-forming units, can be arranged in various orders as known in the art.

A typical multicolour photographic element comprises a support bearing a yellow dye image-forming unit comprised of at least one blue-sensitive silver halide emulsion layer having associated therewith at least one yellow dye-forming coupler, at least one of the yellow dye-forming couplers being a coupler of this invention, and magenta and cyan dye image-forming units comprising at least one green- or red-sensitive silver halide emulsion layer having associated therewith at least one magenta or cyan dye-forming coupler respectively. The element can contain additional layers, such as filter layers.

In the following discussion of suitable materials for use in the emulsions and elements of this invention, reference will be made to Research Disclosure, December 1978, Item 17643, published by Industrial Opportunities Ltd., The Old Harbourmaster's, 8 North Street, Emsworth, Hants P010 7DD, U.K. This publication will be identified hereafter as "Research Disclosure".

The silver halide emulsion employed in the elements of this invention can be either negative-working or positive-working. Suitable emulsions and their preparation are described in Research Disclosure Sections I and II and the publications cited therein. Suitable vehicles for the emulsion layers and other layers of elements of this invention are described in Research Disclosure Section IX and the publications cited therein.

In addition to the couplers of this invention, the elements of the invention can include additional couplers as described in Research Disclosure Section VII, paragraphs D, E, F and G and the publications cited therein. The couplers of this invention and any additional couplers can be incorporated in the elements and emulsions as described in Research Disclosures of Section VII, paragraph C and the publications cited therein.

The photographic elements of this invention or individual layers thereof, can contain brighteners (see Research Disclosure Section V), antifoggants and stabilizers (see Research Disclosure Section VI), antistain agents and image dye stabilizer (see Research Disclosure Section VII, paragraphs I and J), light absorbing and scattering materials (see Research Disclosure Section VIII), hardeners (see Research Disclosure Section XI), plasticizers and lubricants (see Research Disclosure Section XII), antistatic agents (see Research Disclosure Section XIII), matting agents (see Research Disclosure Section XVI) and development modifiers (see Research Disclosure Section XXI).

The photographic elements can be coated on a variety of supports as described in Research Disclosure Section XVII and the references described therein.

Photographic elements can be exposed to actinic radiation, typically in the visible region of the spectrum, to form a latent image as described in Research Disclosure Section XVIII and then processed to form a visible dye image as described in Research Disclosure Section XIX. Processing to form a visible dye image includes the step of contacting the element with a colour developing agent to reduce developable silver halide and oxidize the colour developing agent. Oxidized colour developing agent in turn reacts with the coupler to yield a dye.

Preferred colour developing agents are p-phenylene diamines. Especially preferred are 4-amino-3-methyl-N,N-diethylaniline hydrochloride, 4-amino-3-methyl-N-ethyl-N-β-(methanesulphonamido)ethylaniline sulphate hydrate, 4-amino-3-methyl-N-ethyl-N-β-hydroxyethylaniline sulphate, 4-amino-3-β-(methanesulphonamido)ethyl-N,N-diethylaniline hydrochloride and 4-amino-N-ethyl-N-(2-methoxyethyl)-m-toluidine di-p-toluene sulphonate.

With negative-working silver halide emulsions this processing step leads to a negative image. To obtain a positive (or reversal) image, this step can be preceded by development with a non-chromogenic developing agent to develop exposed silver halide, but not form dye, and then uniform fogging of the element to render unexposed silver halide developable. Alternatively, a direct positive emulsion can be employed to obtain a positive image.

Development is followed by the conventional steps of bleaching, fixing, or bleach-fixing, to remove silver and silver halide, washing and drying.

### Photographic Testing

The methods of photographic testing used in the Examples below are carried out as follows.

### (i) Preparation of Experimental Photographic Coatings

Each coupler of the invention was dissolved in half its weight of di-n-butyl phthalate, with one and a half times its weight of cyclohexanone as auxiliary solvent and dispersed in gelatin. The auxiliary solvent was removed from the dispersion by continuous washing for 6 hours at 4°C and pH 6.0.

Experimental photographic coatings were prepared by coating a cellulose acetate film support with a photosensitive layer comprising a dispersion of the novel coupler as formulated above coated at a laydown of 1.93 mmol/m², a silver bromoiodide emulsion at 0.81 Ag/m² and gelatin at 2.42 g/m². An overcoat containing gelatin at 0.89 g/m² was applied to the photosensitive layer. Bis-vinyl-sulphonylmethane at 1.75% by weight of the total gelatin in the pack was also incorporated into the photosensitive layer. The dried experimental coating was then slit and chopped into 35mm x 12 inch test strips.

Couplers of the invention have also been dispersed with ethyl acetate as auxiliary solvent (subsequently removed by evaporation under reduced pressure) and also in the complete absence of main coupler solvent (NS dispersions) and photographic coatings were prepared as above.

### (ii) Coupler Stability and Crystallinity Measurement

The crystallinity of each coupler dispersion prepared for testing was investigated by spreading a few drops of dispersion on a microscope slide, placing a glass coverslip on top and viewing under a magnification of 1250x using Differential Interference Contrast to enhance the image.

In-film crystallinity of the coupler was assessed largely by visual inspection and deterioration in sensitometry.

In-film stability of the coupler was measured by incubating unexposed test strips for 24 hours at 21°C and 50% relative humidity followed by 1 week dry incubation at 49°C. The strips were then exposed and processed as below and sensitometry compared with that of fresh test strips of the same coupler.

### (iii) Sensitometric Testing

The 35mm test strips were exposed through a 0-4.0 neutral density (ND) step-wedge (0.2 ND step increments) test object and Daylight V, Wratten 35 and 38A and 0.3 ND filters. The strips were processed through a deep-tank sink line at 37.8°C using the following standard process:

| | |
|---|---|
| Colour Developer | 2.5 minutes |
| Bleach (FeIII/EDTA) | 4 minutes |
| Wash | 2 minutes |
| Fix | 4 minutes |
| Wash | 2 minutes |

in which the solutions are those described in the C41 process described in the British Journal of Photography Annual 1977 pages 204-5 in which the colour developing agent was 4-amino-3-methyl-N-ethyl-N-2-hydroxyethylaniline sulphate. The processed strips were then dried to give stepped yellow dye images.

In addition to the above standard conditions test strips were developed in a competing process with the addition of 5.0 g/l citrazinic acid (CZA) to the colour developer solution and adjustment of the pH to 10.0 with sodium carbonate.

For each test strip step-wedge densities were measured using a Macbeth TD504/Hewlett Packard 85 automatic transmission densitometer. Measurements were made of minimum density (Dmin), maximum density (Dmax), contrast (γ), and photographic speed (PS). The ratio of contrast in the CZA competing process to contrast in the standard process (γ_{CZA}/γ_{STD}) is quoted as an indication of in-film reactivity of the coupler.

Silver analysis (X-Ray Fluorescence) of the yellow dye step-wedges produced from a standard process in which the bleach step was omitted enabled silver development curves to be plotted. From these and the D/log E curves were generated Dye Density Yield Curves for each individual coupler. A plot comparing couplers 2 and 3 of the invention with prior art couplers 6 and 7 is shown in Figure 1 of the accompanying drawing.

### (iv) Spectrophotometric Testing

35mm Test strips were exposed as above through a 0-0.3 ND step-wedge (0.1 incremental steps) test object and Daylight V, Wratten 35 and 38A filters and the correct ND filters to give an optical density of about 1.0. The strips were processed using the standard conditions described above and samples cut from the yellow dye image step with density closest to 1.0. Visible absorption spectra (normalized to 1.0 density) were obtained using a Pye Unicam SP8-100 Spectrophotometer. Dye hues are expressed in terms of the wavelength corresponding to the maximum absorption peak (λ max) and the half-bandwidth (HBW) calculated from the spectrophotometric curves.

Extinction coefficients of the yellow dyes were obtained from ethyl acetate solutions of the preformed dyes using a Varian DMS 90/Apple II automated uv/visible spectrophotometer.

### (v) Die Stability Testing

Yellow dye sample patches of density circa 1.0 were prepared as for spectrophotometric testing and their absorption spectra measured as above.

For the dark keeping experiment the yellow dye samples were incubated in a dark oven for periods of 1, 3 and 6 weeks at a constant 60°C and 70% relative humidity. The spectrophotometric curves of the samples were then remeasured and the degree of fade quoted as the fractional decrease in density at the absorption maximum (ΔD) relative to the initial density prior to fading.

### Example 1

The dark/wet fade data for Couplers (1) to (5) are as follows and are compared with comparative compound (6), a commercially used benzoylacetanilide which bears a hydantoin coupling-off group.

| Compound | Dark/wet fade (6 weeks) |
|---|---|
| (1) | 0.06 |
| (2) | 0.04 |
| (3) | 0 |
| (4) | -0.03 |
| (5) | 0.01 |
| (6) (Comparison) | -0.16 |

The structure of Coupler 6 is:
Et herein means ethyl and Bz means benzyl.

It can be seen that dye images formed from all of couplers (1)-(5) of this invention have superior dark/wet stability compared with that of prior art coupler (6).

### Example 2

Table 1, containing examples of the invention (2) and (3), illustrates the superior Dmax and contrast consistently attained in dye images from couplers of the invention relative to a current commercial prior art pivaloylacetanilide coupler (7).

The dark/wet fade data for this set illustrates the superiority of the couplers of the invention (2) and (3) containing a phenolic leaving group over a current commercial benzoylacetanilide (6) which bears a heterocyclic leaving group.

The contrast ratios of this set illustrate the superior activity exhibited by the present benzoylacetanilides relative to the commercial pivaloylacetanilide (7).

## Claims

1. A colour photographic silver halide element comprising a support bearing at least one photographic silver halide emulsion layer and a non-diffusible yellow dye-forming para-R-oxybenzoylacetanilide coupler that has a combination of (a) a para-hydroxyphenylsulphonylphenoxy coupling-off group in the coupling-position, (b) a chloro or trifluoromethyl group in the ortho position on the anilide moiety, and (c) a group on the anilide moiety that is selected from (i) an aliphatic hydrocarbon group that is bonded to the anilide moiety directly or through a linking group that is a carbamoyl (-CONH-), sulphonate (-O-SO₂-), phosphate (-O-PO₂-) or alkylene, (ii) chlorine, and (iii) trifluoromethyl; said anilide moeity having no further substituents; wherein the coupler contains at least one ballast group on at least one of the anilide and para-R-oxybenzoyl moieties; and, wherein R is an unsubstituted or substituted cyclic or non-cyclic aliphatic hydrocarbon group.

2. A colour photographic silver halide element as in Claim 1 wherein the non-diffusible yellow dye-forming coupler is represented by the formula: wherein
R¹ is an unsubstituted or substituted cyclic or non-cyclic aliphatic hydrocarbon group;
Y is chloro or trifluoromethyl;
Z is halogen, trifluoromethyl or -L-R² wherein
R² is an unsubstituted or substituted aliphatic hydrocarbon group,
L is a direct bond or a carbamoyl (-CONH-), sulphonate (-O-SO₂-), phosphate (-O-PO₂-), or alkylene group; and
at least one of R¹ and Z comprises a ballast group.

3. A colour photographic silver halide element as in Claim 2 wherein Z comprises a ballast group and R¹ is alkyl comprising 1 to 4 carbon atoms.

4. A colour photographic silver halide element as in Claim 2 wherein R¹ comprises a ballast group.

5. A colour photographic silver halide element as in Claim 1 wherein the coupler has one of the following structural formulae:

6. A colour photographic silver halide element as in any of Claims 1 to 5 comprising a support bearing at least one red-sensitive silver halide emulsion layer having associated therewith a cyan dye-forming material, at least one green-sensitive silver halide emulsion layer having associated therewith a magenta dye-forming material, and at least one blue-sensitive silver halide emulsion layer having associated therewith said non-diffusible yellow dye-forming coupler.

7. A process of forming a dye image in an exposed colour photographic silver halide element as defined in any of Claims 1 to 6 comprising developing the colour photographic silver halide element in a colour photographic developer.

8. A yellow dye-forming benzoylacetanilide photographic colour coupler as defined in any of claims 1-5.

## Patentansprüche

1. Farbphotographisches Silberhalogenidelement mit einem Träger, auf dem sich mindestens eine photographische Silberhalogenidemulsionsschicht und ein nichtdiffundierender, einen gelben Farbstoff bildender para-R-Oxybenzoylacetanilid-Kuppler befinden, wobei der Kuppler gekennzeichnet ist durch eine Kombination von (a) einer abkuppelnden para-Hydroxyphenylsulfonylphenoxygruppe in der Kupplungsposition, (b) einer Chlor- oder Trifluoromethylgruppe in der ortho-Position an dem Anilidrest, und (c) einer Gruppe an dem Anilidrest, die ausgewählt ist aus (i) einer aliphatischen Kohlenwasserstoffgruppe, die direkt oder über eine Verbindende Gruppe an den Anilidrest gebunden ist, wobei die verbindende Gruppe eine Carbamoyl-(-CONH-), Sulfonat-(-O-SO₂-), Phosphat-(-O-PO₂-) oder Alkylengruppe ist, (ii) Chlor und (iii) Trifluoromethyl; wobei der Anilidrest keine weiteren Substituenten aufweist; wobei der Kuppler mindestens eine Ballastgruppe an mindestens einem der Anilid- und para-R-Oxybenzoylreste aufweist; und, wobei R eine nicht-substituierte oder substituierte cyclische oder nicht-cyclische aliphatische Kohlenwasserstoffgruppe ist.

2. Farbphotographisches Silberhalogenidelement nach Anspruch 1, in dem der nicht-diffundierende einen gelben Farbstoff bildende Kuppler durch die folgende Formel wiedergegeben wird: worin bedeuten:
R¹ eine unsubstituierte oder substituierte cyclische oder nicht-cyclische aliphatische Kohlenwasserstoffgruppe;
Y Chlor oder Trifluoromethyl;
Z Halogen, Trifluoromethyl oder -L-R², wobei
R² eine unsubstituierte oder substituierte aliphatische Kohlenwasserstoffgruppe ist,
L eine direkte Bindung oder eine Carbamoyl-(-CONH-), Sulfonat-(-O-SO₂-), Phosphat-(-O-PO₂-) oder Alkylengruppe und
mindestens einer der Reste R¹ und Z eine Ballastgruppe.

3. Farbphotographisches Silberhalogenidelement nach Anspruch 2, in dem Z eine Ballastgruppe darstellt, und R¹ eine Alkylgruppe mit 1 bis 4 Kohlenstoffatomen.

4. Farbphotographisches Silberhalogenidelement nach Anspruch 2, in dem R¹ eine Ballastgruppe darstellt.

5. Farbphotographisches Silberhalogenidelement nach Anspruch 1, in dem der Kuppler einer der folgenden Strukturformeln entspricht:

6. Farbphotographisches Silberhalogenidelement nach einem der Ansprüche 1 bis 5 mit einem Träger, auf dem sich mindestens eine rotempfindliche Silberhalogenidemulsionsschicht, der ein einen blaugrünen Farbstoff bildendes Material zugeordnet ist, mindestens eine grünempfindliche Silberhalogenidemulsionsschicht, der ein einen purpurroten Farbstoff bildendes Material zugeordnet ist und mindestens eine blauempfindliche Silberhalogenidemulsionsschicht, der der nicht-diffundierende, einen gelben Farbstoff bildende Kuppler zugeordnet ist, befinden.

7. Verfahren zur Herstellung eines Farbstoffbildes in einem exponierten farbphotographischen Silberhalogenidelement nach einem der Ansprüche 1 bis 6, bei dem das farbphotographische Silberhalogenidelement in einem farbphotographischen Entwickler entwickelt wird.

8. Ein einen gelben Farbstoff bildender photographischer Benzoylacetanilid-Farbkuppler nach einem der Ansprüche 1 bis 5.

## Revendications

1. Produit aux halogénures d'argent pour la photographie en couleurs comprenant un support avec, sur ce support, au moins une couche d'émulsion photographique aux halogénures d'argent, et un coupleur para-R-oxybenzoylacétanilide formateur de colorant jaune non-diffusible qui combine (a) un groupe parahydroxyphénylsulphonylphénoxy se séparant par couplage dans la position de couplage, (b) un groupe chloro ou trifluorométhyle en position ortho sur le radical anilide, et (c) sur le radical anilide, un groupe choisi parmi (i) les groupes hydrocarbonés aliphatiques liés au radical anilide directement ou par l'intermédiaire d'un groupe de liaison carbamoyle (-CONH-), sulfonate (-O-SO₂-), phosphate (-O-PO₂-) ou alkylène, (ii), le chlore et (iii) le radical trifluorométhyle ; ce radical anilide n'ayant aucun autre substituant ; le coupleur contenant au moins un groupe de lestage sur au moins l'un des radicaux anilide ou para-R-oxybenzoyle ; R étant un groupe hydrocarboné aliphatique cyclique ou non cyclique, substitué ou non substitué.

2. Produit aux halogénures d'argent pour la photographie en couleurs selon la revendication 1, dans lequel le coupleur formateur de colorant jaune non diffusible est représenté par la formule : où
R¹ est un groupe hydrocarboné aliphatique, cyclique ou non-cyclique, substitué ou non substitué ;
Y est chloro ou trifluorométhyle
Z est halogène, trifluorométhyle ou -L-R² dans lequel
R² est un groupe hydrocarboné aliphatique ou non substitué ;
L est une liaison directe ou un groupe carbamoyle (-CONH-), sulfonate (-O-SO₂-), phosphate (-O-PO₂) ou alkylène et,
au moins l'un des groupes R¹ et Z comprend un groupe de lestage.

3. Produit aux halogénures d'argent pour la photographie en couleurs selon la revendication 2, dans lequel Z comprend un groupe de lestage et R¹ est alkyl comprenant de 1 à 4 atomes de carbone.

4. Produit aux halogénures d'argent pour la photographie en couleurs selon la revendication 2, dans lequel R¹ comprend un groupe de lestage.

5. Produit aux halogénures d'argent pour la photographie en couleurs selon la revendication 1, dans lequel le coupleur présente l'une des formules suivantes :

6. Produit aux halogénures d'argent pour la photographie en couleurs selon l'une des revendications 1 à 5 comprenant un support portant au moins une couche d'émulsion aux halogénures d'argent sensible au rouge associée à un coupleur formateur de colorant cyan, au moins une couche d'émulsion aux halogénures d'argent sensible au vert associée à un coupleur formateur de colorant magenta et au moins une couche d'émulsion aux halogénures d'argent sensible au bleu associée audit coupleur formateur de colorant jaune non diffusible.

7. Procédé pour former une image de colorant dans un produit aux halogénures d'argent pour la photographie en couleur selon l'une des revendications 1 à 6, préalablement exposé, comprenant le développement de ce produit dans un révélateur pour la photographie en couleur.

8. Coupleur benzoylacétanilide formateur de colorant jaune pour la photographie en couleur tel que défini dans l'une des revendications 1-5.
